

# UNITED STATES PATENT OFFICE.

JAMES H. HOLLEN, OF LANSINGBURG, NEW YORK.

## MIXED PAINT.

SPECIFICATION forming part of Letters Patent No. 341,576, dated May 11, 1886.

Application filed February 17, 1886. Serial No. 192,442. (No specimens.)

*To all whom it may concern:*

Be it known that I, JAMES H. HOLLEN, a citizen of the United States, residing at Lansingburg, in the county of Rensselaer and State 5 of New York, have invented a new and useful composition to be used as a liquid filler and finisher for filling and impregnating the pores or surface interstices of fine dressed hard woods used for interior and exterior building 10 and decorative purposes, and for articles of domestic and office furniture, wainscoting, dados, and panels, and for finishing and developing the grain of such woods on the surfaces thereof, of which the following is a specification.

My composition consists of the following ingredients combined, preferably, in the proportions stated, viz: bleached gum-shellac, three pounds; corn-starch, one pound; pulverized 20 magnesia, one-half pound; pulverized steatite, one-half pound; alcohol, one and one-half gallon.

This composition is prepared for use by first cutting or dissolving the gum-shellac in 25 the alcohol, then adding the corn-starch, pulverized magnesia, and pulverized steatite into the mixture in the order named, and thoroughly agitating the whole over a slow fire until a liquid is formed of a consistence to 30 flow freely and spread evenly on and penetrate readily the surface of the wood to be treated, when applied by means of an ordinary varnish-brush.

In using and applying the above-named composition in practice the following method is 35 preferably to be observed: Spread the "liquid filler and finisher" over the surface of the wood or wood-work to be filled and impregnated in the same manner as varnish is applied with a 40 varnish-brush; then allow the work to stand from four to five hours until the liquid filler and finisher shall have become thoroughly set and impregnated into the pores and interstices of the surface grain of the wood; then, 45 when the work has become set, sand-paper it slightly, and finish with one coat of varnish or oil-finish.

The utility and novelty of my invention is that by the use of the above-named composition—liquid filler and finisher—the surface-interstices of the woods to be treated are thor-

oughly and expeditiously filled and impregnated at a great saving of labor over the methods and by the means heretofore employed for treating woods with that object in view. The 55 natural beauties and delicate traceries of the grain of such fine-grained woods as satin-wood, ash, butternut, walnut, cherry, maple, and the like are brought out more clearly and fully to the eye, and the general effect of the work 60 is heightened and beautified.

By the omission of the pulverized steatite in the above composition the liquid forms a finish of itself without the oil or varnish finish; but in such case requires two or more coats or 65 applications to form a smooth polished surface on the woods or work.

I am aware that painters, decorators, and wood-finishers have heretofore used compositions consisting of two or more of the above-named ingredients, omitting some one or more of the others, to form a viscid glutinous paste for the purpose of filling or stuffing the pores and surface-interstices of fine, dressed, hard woods as a foundation to receive an additional 70 finish, which paste is required to be slowly and laboriously rubbed in and upon the surfaces of such woods by means of cloths or with the bare hands, and requiring afterward to be slowly and laboriously scraped off and 75 smoothed to remove the inequalities of the paste; but I am not aware that all of the ingredients of my composition in the proportions stated or otherwise have been used together to form a liquid, so as to be applied by means 80 of a brush, and to flow freely and to impregnate equally and thoroughly the interstices on the surfaces of such woods as described, and to bring out and develop the grain thereof in 85 a quick and labor-saving manner.

What I claim, and desire to secure by Letters Patent of the United States, is—

The herein-described wood filler and finisher, consisting of bleached gum-shellac, corn-starch, pulverized magnesia, pulverized steatite, and alcohol, combined in about the 90 proportions herein specified.

JAMES H. HOLLEN.

Witnesses:

JEREMIAH K. LONG,  
JOHN D. COLBY.